

## UNITED STATES PATENT OFFICE.

HENRY S. MARSH AND RALF S. COCHRAN, OF YOUNGSTOWN, OHIO, ASSIGNEES TO AMERICAN COPPERAS COMPANY, OF YOUNGSTOWN, OHIO, A CORPORATION OF DELAWARE.

## PICKLING.

No Drawing.

Application filed November 14, 1924. Serial No. 749,981.

*To all whom it may concern:*

Be it known that we, HENRY S. MARSH and RALF S. COCHRAN, residing at Youngstown, in the county of Mahoning and State 5 of Ohio, both citizens of the United States, have invented or discovered certain new and useful Improvements in Pickling, of which improvements the following is a specification.

10 Our invention relates to improvements in the method of pickling ferrous articles, particularly rolled steel sheets and plates, and its objects are the production of clean surfaces, and also the overcoming of conditions which tend to delay and prolong 15 the normal operation of pickling.

In the practice of pickling rolled steel sheets and plates, the articles are apt to come from the pickling vat, not bright and white, as they should be, but clouded and mottled and streaked with dull brown. A sheet or plate so discolored is, because of its very appearance, less acceptable to the customer, and, furthermore, it is in some 25 respects inferior in utility and serviceability. For instance, the scrap cut from the sheets or plates in their further fabrication, is commonly fashioned to other articles. The articles so produced are sometimes found to 30 be defective, in that they are not responsive to the case-hardening operation.

We have investigated, and have discovered that the mottled and darkened appearance upon the surfaces of the sheets and plates, 35 is due to the presence of other metals, chiefly copper, and, in less degree, arsenic and lead, electroplated upon or otherwise deposited upon the steel surfaces while in the pickling bath.

40 Copper has of late years been increasingly used as an alloy of iron, and this, together with the circumstances that steel parts are in industry generally, often provided with copper fittings of one sort and another, results in this: that steel scrap contains a very appreciable, though very uncertain, copper content. In steel-making steel scrap is charged together with pig iron into the refining furnace, and in consequence 45 copper appears as an appreciable ingredient of the newly produced steel.

In the preparation of the pickling bath, too, and in the reclaiming of spent pickling solutions, the dilute acid which constitutes

the bath in its essence, is apt to carry some 55 small quantity of copper salt, derived from containers and conveyors with which it has come into contact. The raw acid, as now found on the market, is likely to contain arsenic and lead in small quantities. 60

When under such conditions the pickling operation is performed upon steel sheets and plates, two undesirable circumstances appear: first, the sheets and plates are apt to come from the bath mottled and dirty 65 in appearance, as has been said. This we impute primarily to the presence of copper, and in less degree to lead and arsenic. In the second place, the operation of pickling is retarded, and this we impute primarily to the presence of lead and arsenic, 70 which act as inhibitors, and in less degree to copper.

The pickling solution, attacking the surface of the sheet, tends to eat away the copper as well as the iron, but there is a countervailing tendency of the copper salt in solution (copper sulphate, ordinarily), whether initially present in the bath, or derived from the material under treatment, 75 to break up; the phenomenon of electrolysis appears, and metallic copper is deposited electrolytically upon the surface of the steel sheet or plate. The dull and dirty appearance of this deposit is due to the condition 80 of the electrolyte, and particularly to the presence of other metals or metalloids, deposited with the copper.

We have discovered, and herein lies our invention, that by generating in the pickling 85 bath and in sufficient quantities, sulphuretted hydrogen, the copper present in the bath, from whatever source derived and in whatever condition, and such other metals and metalloids as arsenic and lead, will combine or recombine to form metallic sulphides, and in the form of metallic sulphides these undesired metals will be eliminated, the electrolytic deposits will not occur, nor will the normal pickling operation 90 be retarded.

In the practice of our invention we preferably begin with the pickling liquid reclaimed from previous service. We bring this pickling liquid into a suitable tank or 105 container, where we introduce into it iron sulphide. The acid reacts upon the iron sulphide and produces sulphuretted hydro-

gen; the sulphuretted hydrogen reacts upon the salts of the undesired metals and forms sulphides of those metals. These metallic sulphides are insoluble, and we allow them 5 to settle and separate them, and introduce the liquid into the pickling vat freed from them. In this operation of separating the undesired metallic sulphides we accelerate separation by increasing the temperature 10 of the liquid to approximately 120° F. And this we conveniently accomplish by the injection of steam into the liquid.

Proceeding to the pickling operation itself, we introduce iron sulphide into the 15 pickling vat also. And there also the acid reacting upon the iron sulphide releases sulphuretted hydrogen. And the sulphuretted hydrogen in turn, reacting with the copper as it is eaten by the acid from the sheets or 20 plates under treatment, forms copper sulphide, and in that ultimate form the copper is eliminated from the further reactions, and held from electrolytic deposition. Similarly there is no deposit of other undesired 25 metal, and the sheets and plates go from the bath with the desired bright and clean surfaces.

In order to make our invention effective to the fullest extent, it is desirable that the 30 pickling bath be at all times saturated with sulphuretted hydrogen. This is a condition which in practice is not difficult to maintain; all that is requisite is that the iron sulphide be supplied in such quantity that 35 the bath smells of sulphuretted hydrogen. The relatively high temperature normally maintained in pickling tends of course to release whatever sulphuretted hydrogen may be present in solution. In order therefore 40 to insure the presence of the sulphuretted hydrogen in sufficient quantities, we maintain within the pickling vat good-sized lumps of iron sulphide. From these the

sulphuretted hydrogen is generated gradually, and as it is generated it is taken up 45 continuously by the bath.

It remains only to say that in the case of sheets of light gauge, sheets such as have been rolled and annealed in packs, and which present relatively large and clean 50 surfaces to the action of the liquid, we have found the difficulty less, to the correction of which our invention is addressed. But in the case of heavier sheets and plates, and in case the coatings of oxide are continuous 55 and heavy, we are able in the practice of our invention to overcome a difficulty of substantial magnitude and achieve a substantial gain.

We claim as our invention:

1. The method herein described of pickling metallic objects which consists in conducting the pickling operation in a pickling solution burdened with sulphuretted hydrogen.

2. The method herein described of producing bright-surfaced pickled articles of adulterated iron which consists in conducting the pickling operation in a pickling bath saturated with sulphuretted hydrogen.

3. The method herein described of conducting the pickling operation upon metallic objects which consists in causing reclaimed pickling solution at elevated temperature to react upon iron sulphide, allowing the precipitate to settle, and introducing the articles to be pickled into the solution so previously treated.

4. A pickling bath consisting of a body of dilute sulphuric acid having immersed in it lumps of iron sulphide.

In testimony whereof we have hereunto set our hands.

HENRY S. MARSH.  
RALF S. COCHRAN.